

1

2,975,137

## COMPRESSION REFRIGERATION WORKING FLUID

Archibald P. Stuart, Media, Pa., assignor to Sun Oil Company, Philadelphia, Pa., a corporation of New Jersey

No Drawing. Filed Dec. 30, 1955, Ser. No. 556,448

10 Claims. (Cl. 252—68)

This invention relates to an improved compression refrigeration working fluid comprising a halogen-substituted hydrocarbon refrigerant, a mineral oil lubricant, and a copper plating inhibiting amount of a group IV-B organo-metallic compound.

In compression refrigeration systems which employ a halogen-substituted hydrocarbon refrigerant and a mineral oil lubricant, copper plating is an important problem. Copper is removed from parts of the refrigeration apparatus which are formed of this metal, e.g., heat exchanger tubes, and the removed copper is transported to non-copper parts of the system, especially ferrous parts, where it is deposited as a layer or plate. Moving parts of the system which continually require lubrication such as compressor parts are particularly susceptible to copper plating. The copper plating increases wear of moving parts and causes operational difficulties and even failure of refrigeration systems.

Now in accordance with the present invention, there is incorporated in the compression refrigeration working mixture of halogen-substituted hydrocarbon refrigerant and mineral oil lubricant a copper plating inhibiting amount of a group IV-B organo-metallic compound. Compounds which have been found to be effective copper plating inhibitors and which are used in this invention are compounds having the structural formula:



or



where M is tin, lead or germanium, R<sub>1</sub>, R<sub>2</sub>, R<sub>3</sub> and R<sub>4</sub> are hydrocarbon radicals, hydrocarboxy radicals or carboxylic acid radicals and R<sub>5</sub> is a hydrocarbonyloxy radical or a dicarboxylic acid radical.

It is preferred to use organo-tin compounds in the practice of this invention since organo-tin compounds are generally better copper plating inhibitors than organo-germanium and organo-lead compounds. However, organo-germanium and organo-lead compounds are also effective copper plating inhibitors and can be used in the practice of the present invention.

The group IV-B organo-metallic copper plating inhibitors used in the invention preferably have at least one substituent which is a hydrocarboxy radical, a hydrocarbonyloxy radical, a carboxylic acid radical or a dicarboxylic acid radical. It has been found that these compounds are somewhat more effective in suppressing copper plating than are group IV-B organo-metallic compounds having all hydrocarbon substituents although these latter compounds can be used to suppress copper plating in this invention. Copper plating inhibitors of the invention which do not have a hydrocarbonyloxy or a dicarboxylic acid substituent radical preferably have two or three hydrocarboxy or carboxylic radical substituents. The presence of a hydrocarbon substituent is believed to impart high solubility in the refrigerator working fluid to the additives of this invention, and accordingly the ad-

2

ditives preferably contain at least one hydrocarbon radical substituent.

The hydrocarbon substituent radicals on the copper plating inhibitors of the invention are normal, branched chain or cyclic hydrocarbon radicals. Aliphatic, alicyclic or aromatic radicals are suitable. It is preferred that the aliphatic and alicyclic substituent radicals are saturated although inhibitors with unsaturated aliphatic and alicyclic substituent radicals can be used. Preferred hydrocarbon radicals are those having about 1 to 20 carbon atoms per radical. Examples of specific hydrocarbon radicals which are suitable substituents on the copper plating inhibitors of this invention are methyl, ethyl, propyl, butyl, amyl, cyclohexyl, dodecyl, 1-butetyl, cyclohexenyl, cyclopentyl, isobutyl, isopropyl, benzyl, phenyl, tolyl, xylyl, cumyl, cymyl, pseudocumyl, naphthyl, anthryl, phenanthryl and the like.

The organo-metallic inhibitors' hydrocarboxy substituent radicals are any of the above described hydrocarbon radicals connected by an oxygen atom to the metal atom of the organo-metallic compound. Preferred molecular size of the hydrocarboxy radical substituents is about 1 to 20 carbon atoms. Specific examples of suitable substituent hydrocarboxy radicals are methoxy, ethoxy, propoxy, isopropoxy, butoxy, cyclopentoxy, cyclohexoxy, benzyloxy, phenoxy, toloxy and the like.

The carboxylic acid substituents on the copper plating inhibitors of the invention are any of the above described hydrocarbon radicals connected by

30

$$\begin{array}{c} O \\ \diagup \\ -C=O- \end{array}$$

to the metal atom of the inhibitor. Preferred molecular size of the carboxylic acid substituents is about 2-21 carbon atoms. Specific examples of suitable carboxylic acid substituent radicals are acetic, propionic, butyric, lauric, stearic, naphthenic, benzoic, hexahydrobenzoic, isobutyric, isovaleric, 3-butenoic, senecioic acid radicals and the like.

The copper plating inhibitors used in the invention can 40 be dicarboxylic acid substituted compounds or hydrocarbonyloxy substituted compounds. The dicarboxylic acid or hydrocarbonyloxy substituent radicals are illustrated by R<sub>5</sub> in the above structural formula. The dicarboxylic acid substituent comprises a hydrocarbon connected by

45 two

$$\begin{array}{c} O \\ \diagup \\ -C=O- \end{array}$$

groups to the metal atom of the organo-metallic compound. The hydrocarbonyloxy substituent comprises a hydrocarbon connected by two oxygen atoms to the metal atom of the organo-metallic compound. The hydrocarbon portion of the hydrocarbonyloxy and dicarboxylic acid substituents can be aromatic or it can be saturated 55 or unsaturated aliphatic or alicyclic. It is preferred that the hydrocarbon portion of the dicarboxylic acid and hydrocarbonyloxy substituents have a molecular size of about 2 to 10 carbon atoms. Specific examples of suitable hydrocarbonyloxy substituent radicals are ethylene-60 dioxy, 1,2-propylenedioxy, 1,3-propylenedioxy, 1,2-butyl-enedioxy, 1,3-butylenedioxy, 1,4-butylenedioxy, 1,4-dioxy, 2-butene, 1,2-dioxy benzene, 1,3-cyclohexylenedioxy radicals and the like. Specific examples of suitable dicarboxylic acid radicals are maleic, 1,2-benzenedicarboxylic, malonic, 1,2-cyclohexandicarboxylic, phthalic acid radicals and the like.

Examples of group IV-B organo-metallic compounds which can be used in carrying out the present invention are tetraethyl germanium, di-n-butyltin diacetate, di-n-butyltin dilaurate, tetra-p-tolyltin, di-n-butyltin maleate, di-n-butyl dibutoxy tin, di-n-butyl ethylenedioxy tin, di-n-butyltin phthalate, 1,4-dioxy 2-butene tin, tetraethyl

lead and the like. The use of di-n-butylin diacetate, di-n-butylin dilaurate, di-n-butylin maleate, di-n-butoxy tin, di-n-butyl ethylenedioxy tin, di-n-butylin phthalate and 1,4-dioxy 2-butene tin is especially preferred.

The halogen-substituted hydrocarbon refrigerants which form a part of the improved working fluids of this invention can be any of the halogen-substituted hydrocarbons conventionally used as refrigerants in compression refrigeration systems. Examples of these refrigerants are dichlorodifluoromethane, 1,2-dichloro-1, 1,2,2-tetrafluoroethane, dichloromonofluoromethane, monochlorodifluoromethane, trichloromonofluoromethane, 1,1,2-trichloro-1, 2,2-trifluoroethane and the like.

The mineral oil lubricant which forms part of the novel working fluid of the invention can be any conventional compression refrigeration mineral oil lubricant. Such oils generally have viscosities in the range of 75 to 500 SUS @ 100° F., pour points of -15° F. to -50° F., low floc points and do not vaporize at conditions in the refrigeration system.

It is necessary according to the present invention to incorporate sufficient of the organo-metallic compound in the lubricant-refrigerant mixture to inhibit copper plating in the refrigeration system. Generally the use of amounts of the organo-metallic copper plating inhibitor in the range of 0.01% to 2% by weight of the lubricant is sufficient to effectively suppress copper plating. However, amounts outside this range can, on occasion, be successfully used.

The following illustrates a practice of the present invention:

Di-n-butylin maleate is added to a compression refrigeration working fluid comprising dichlorodifluoromethane refrigerant and mineral oil lubricant. The di-n-butylin maleate is used in amount of 0.5% of the lubricant. This resulting mixture when used as working fluid in a compression refrigeration system, effectively suppresses copper plating in the system.

#### Example

The effectiveness of refrigerator working fluid additives of this invention as copper plating inhibitors was tested in the following way. Minor amounts of the inhibitors were added to different portions of a mixture comprising about 50% of carbon tetrachloride and 50% of a naphthenic-base distillate refrigerator lubricating oil. The oil had been furfural-refined, acid treated, and clay treated; the oil had an API gravity of about 24.4 and a S.U. viscosity at 100° F. of about 160 seconds. A copper-steel coupling was suspended in each mixture, and each mixture was maintained for extended periods of time at 150° F. At the end of the test period, the steel surface was examined to determine the percent of the steel surface on which copper had been deposited. The following table shows the results obtained with inhibitors of this invention as compared to a control sample having no inhibitor:

| Sample  | Inhibitor              | Inhibitor Amt., Wt. Percent of Oil | Test Period, Hours | Percent of Surface Plated |
|---------|------------------------|------------------------------------|--------------------|---------------------------|
| Control |                        |                                    |                    |                           |
| 1.....  | di-n-butylin dilaurate | 0.5                                | 72                 | 80                        |
| 1.....  | do                     | 0.5                                | 220                | 0                         |
| 2.....  | di-n-butylin diacetate | 0.4                                | 288                | 100                       |
| 2.....  | do                     | 0.4                                | 504                | slight stain              |
| 3.....  | di-n-butylin maleate   | 0.45                               | 1,000              | 0                         |

These results show that the organo-metallic additives of this invention are effective suppressors of copper plating. Of the additives tested, dibutyltin maleate gave somewhat better results than dibutyltin dilaurate or dibutyltin diacetate.

I claim:

1. A compression refrigeration working fluid consist-

ing essentially of a halogen-substituted hydrocarbon refrigerant, a lubricating amount of a mineral oil lubricant and a copper-plating inhibiting amount of an organo-tin compound having a structural formula selected from the group consisting of:



10 and



wherein:  $R_1$  is a 1 to 20 carbon atom hydrocarbon radical selected from the group consisting of: alkyl, cycloalkyl, alkaryl and aryl radicals;  $R_3$  is a radical selected from the group consisting of  $-OR_1$  and



wherein  $R_1$  is as defined above;  $R_2$  and  $R_4$  are radicals each selected from the group consisting of  $R_1$ ,  $-OR_1$  and



wherein  $R_1$  is as defined above; and  $R_5$  is a radical having 2 to 10 carbon atoms and is selected from the group consisting of hydrocarbonyloxy and dicarboxylic acid radicals wherein the hydrocarbon portion is selected from the group consisting of aliphatic, alicyclic and aromatic portions.

2. A composition according to claim 1 wherein  $R_3$  is a hydrocarbonyloxy radical.

3. A composition according to claim 1 wherein  $R_3$  is a carboxylic acid radical.

4. Composition according to claim 1 wherein said organo-tin compound is present in an amount equal to between 0.01 and 2.0 wt. percent of the mineral oil lubricant present in said compression refrigeration working fluid.

5. A compression refrigeration working fluid consisting essentially of a halogen-substituted hydrocarbon refrigerant, a lubricating amount of a mineral oil lubricant and a copper-plating inhibiting amount of an organo-tin compound selected from the group consisting of di-n-butylin diacetate; di-n-butylin dilaurate; di-n-butylin maleate; di-n-butyl dibutoxy tin; di-n-butyl ethylenedioxy tin; di-n-butylin phthalate; and 1,4-dioxy 2-butene tin.

6. A composition according to claim 5 wherein said organo-tin compound is di-n-butyl dibutoxy tin.

7. A composition according to claim 5 wherein said organo-tin compound is di-n-butylin diacetate.

8. A composition according to claim 5 wherein said organo-tin compound is di-n-butylin dilaurate.

9. A composition according to claim 5 wherein said organo-tin compound is di-n-butyl ethylenedioxy tin.

10. A composition according to claim 5 wherein said organo-tin compound is di-n-butylin maleate.

#### References Cited in the file of this patent

#### UNITED STATES PATENTS

|           |              |                |
|-----------|--------------|----------------|
| 1,966,881 | Braunn       | July 17, 1934  |
| 2,060,728 | Fleischer    | Nov. 10, 1936  |
| 2,288,288 | Lincoln      | June 30, 1942  |
| 2,421,631 | Lincoln      | June 3, 1947   |
| 2,468,544 | Clark        | Apr. 26, 1949  |
| 2,493,213 | Altamura     | Jan. 3, 1950   |
| 2,523,863 | Cook         | Sept. 26, 1950 |
| 2,578,359 | Jenkins      | Dec. 11, 1951  |
| 2,789,105 | Tamka et al. | Apr. 16, 1957  |

#### FOREIGN PATENTS

Great Britain Jan. 27, 1954